

## UNITED STATES PATENT OFFICE

1,920,921

## ARC CARBON

Merrill J. Dorcas, Cleveland, Ohio, assignor to  
National Carbon Company, Inc., a Corporation  
of New York

No Drawing. Application January 27, 1928  
Serial No. 250,069

2 Claims. (Cl. 176—134)

This invention relates to electrodes for arc lamps and especially to electrodes which are adapted for use with a high intensity arc to produce a light having a color value similar to that of an incandescent lamp.

When a direct current arc, the positive electrode of which consists of a cored arc carbon, is operated above a certain critical current density two related effects are produced, a relatively deep crater is formed and there is in this crater an incandescent gas ball of extremely high intrinsic brilliancy. This effect is termed "the high intensity effect" and the current density required to produce it is a function of the diameter of the carbon and the composition of the core. Hitherto it has been supposed that it was impossible to produce color changes in the high intensity arc by varying the electrode composition. This belief was based in part on theoretical considerations and in part upon actual experiment. I have found, however, that this belief is incorrect and that the color value of the light emitted from a high intensity arc, is capable of modification by the use of suitable addition agents in the core of the positive electrode. Such addition agents are the compounds of calcium and strontium. While various salts of these elements may be used I have found the halides, particularly the fluorides, well adapted for this purpose.

These addition agents are especially suitable for this use as by properly proportioning the same it is possible to obtain light from a high intensity arc which has a color value similar to that emitted from an incandescent tungsten light. It is desirable to obtain such color values, not only for the purpose of producing a light such as people are accustomed to, but also for use in the projection of colored moving pictures and the taking of pictures whether for still or motion picture work. In the colored motion picture process the color effect is obtained by either the additive or subtractive method. In either case two or more colors, usually red and green, are used and it is difficult to obtain natural colors for other than the pure reds and greens or other colors used. Various compromises have to be effected and these naturally vary with variations in the color value of the light used in projection. Because large numbers of projectors using incandescent tungsten lights or the incandescent crater of a carbon arc as the light source are in use, the manufacturers have based their process upon this light and a light source having any other color value gives an incorrect color render-

ing. I have found that in projections over long distances, such as are found in the larger theaters of the present time, these lights do not give a sufficient intensity and it is desirable to use a high intensity arc. This is not feasible with the present high intensity arc for the reasons already stated. If the change were made color films now extant could not be used with the high intensity projectors and a new process would have to be worked out to make special films for them. The special films would however be unsuitable for the smaller theaters which use incandescent lamps in their projectors. By modifying the color value of the light from the high-intensity arc so that it approximates that of the incandescent lamp I have avoided this difficulty.

Similarly in the taking of pictures, not only still, but more especially motion pictures, a panchromatic film is used. This film is sensitized with an emulsion containing dyes which render the emulsion sensitive to lights of varying colors in such a manner that the black and white image produced in the positive gives a rendering which approximates that given by the human eye. The present panchromatic films give fairly good results if the illumination is provided by an incandescent source such as a tungsten incandescent bulb or the incandescent crater of a suitable carbon arc and in order to use the high intensity arc for lighting objects to be photographed it was necessary either to modify the color value of the high intensity arc or to work out a new emulsion for panchromatic films. By this invention I have succeeded in modifying the high intensity arc light to give a color value similar to that of the incandescent tungsten light.

While I have found the carbon electrodes produced in accordance with my invention to be of especial value in connection with high intensity arcs, they are also adapted for use with current densities below those which produce the high intensity effect described above with both direct and alternating current.

In order to produce a modified high intensity arc light I form the positive carbons with a core containing calcium and strontium. While various cores may be used I have found the following composition satisfactory: calcium fluoride 40 parts, strontium fluoride 10 parts, sodium or potassium silicate 5 parts, carbon flour 45 parts, tar sufficient to bind. In a particular instance a positive 11 millimeters in diameter was provided with a core of this composition having a diameter of approximately 5.5 millimeters and operated with a negative approximately 9

mm. in diameter. At 75 to 200 amperes the high intensity effect was obtained, and the color value was a sufficiently close approximation to that of an incandescent lamp.

intensity arc in which approximately half the core is composed of fluoride salts of calcium and strontium in a ratio of substantially 40 parts of calcium fluoride to 10 parts of strontium fluoride, the carbon electrode being characterized by the fact that, when burned as the positive electrode in an arc of high intensity, the arc has a color value similar to that of an incandescent light.

80

5 I claim:

1. A core for carbon electrodes comprising calcium fluoride 40 parts, strontium fluoride 10 parts, sodium or potassium silicate 5 parts, carbon flour 45 parts, and tar sufficient to bind.

10 2. A cored carbon electrode for use in a high

MERRILL J. DORCAS.

85

15

90

20

95

25

100

30

105

35

110

40

115

45

120

50

125

55

130

60

135

65

140

70

145

75

150